# EUROPEAN PATENT SPECIFICATION

(11) **EP 1 270 807 B1**
(45) Date of publication and mention of the grant of the patent: **11.01.2006**
(21) Application number: 02013714.7
(22) Date of filing: 20.06.2002
(51) Int. Cl.: D21F 5/00, D21F 7/10, D03D 3/04

(54) **Pin seamed papermaker's press felt with laminated base fabric having low melt material machine directions yarns**
Papiermacherfilz mit Doppelösennaht und laminiertem Grundgewebe welches niedrig schmelzende Kettfäden enthält
Feutre de presse de machine à papier agraffé par broche et comprenant des files de chaine de matériau fusible à basse température dans le tissu stratifié

(30) Priority: 20.06.2001 US 885430
(43) Date of publication of application: 02.01.2003
(73) Proprietor: WEAVEXX CORPORATION, Wake Forest, North Carolina 27588 (US)
(72) Inventor: Marchand, Rene, Fayetteville, Georgia 30215 (US)
(74) Representative: Popp, Eugen

(56) References cited:
- WO-A-00/17433
- US-A- 5 897 745

## Description

### Field of the Invention

The present invention relates generally to papermaking, and more particularly to fabrics used in papermaking.

### Background of the Invention

In the conventional fourdrinier papermaking process, a water slurry, or suspension, of cellulosic fibers (known as the paper "stock") is fed onto the top of the upper run of an endless belt of woven wire and/or synthetic material that travels between two or more rollers. The belt, often referred to as a "forming fabric," provides a papermaking surface on the upper surface of its upper run which operates as a filter to separate the cellulosic fibers of the paper stock from the aqueous medium, thereby forming a wet paper web. The aqueous medium drains through mesh openings of the forming fabric, known as drainage holes, by gravity alone or with assistance from one or more suction boxes located on the lower surface (i.e., the "machine side") of the upper run of the fabric.

After leaving the forming section, the paper web is transferred to a press section of the paper machine, in which it is passed through the nips of one or more pairs of pressure rollers covered with another fabric, typically referred to as a "press felt." Pressure from the rollers removes additional moisture from the web; the moisture removal is often enhanced by the presence of a "batt" layer on the press felt. The paper is then conveyed to a drier section for further moisture removal. After drying, the paper is ready for secondary processing and packaging.

Press felts typically include one or more base fabric layers; these can be "flat-woven" and formed after weaving into an endless belt, or can be woven in endless form. Generally, the flat-woven process is preferred, as it is typically less expensive and more versatile than the endless weaving process. Also, in many instances the felt is cut widthwise and reattached to simplify installation on a paper machine, in which case some of the advantages of endless weaving (such as the absence of a seam in the fabric) are lost.

Of course, flat weaving a fabric of a base layer requires that provision be made for joining it into endless belts. Such joints should be constructed in such a manner that they are Sufficiently strong to withstand the extreme load, temperature, and wear conditions the press felt experiences, yet do not cause the surface of the press felt above the seam to unduly mark the paper. One popular method of joining the base fabric of a press felt is to form loops with machine direction yarns on each end of the base fabric. To form the flat-woven base fabric into an endless belt, the ends of the fabric are placed adjacent to each other, with each of the loops on one end positioned between two loops on the other end in interdigitating fashion. A "pin" (usually formed of mutilfilament polymeric fiber strands) is then inserted into all of the loops to join the ends. After the batt layer(s) are needled or otherwise attached to the base layer, the batt layer(s) are cut at the seam location, the pin is removed, and the finished press felt is shipped to a paper mill. Once at the paper mill, the press felt can be installed by placing it onto a paper machine, then inserting another (usually more flexible) multifilament pin into the loops. Examples of this type of seam are described in U.S. Patent Nos. 4, 764,417 and 4,737,241 to Gulya, 4,601,785 to Lilja et al., and 5,476,123 to Rydin.

In some press felts, the base fabric layer itself contains multiple fabric layers (i.e., is a "laminated" base layer). For example, a felt may contain a "duplex" fabric (i.e., a fabric having upper and lower sets of machine direction yams interwoven with at least one set of cross machine direction yarns - also known as a "double layer" fabric) as well as a finer mesh single layer fabric (i.e., a fabric having only one set each of machine direction yarns and cross machine direction yarns). This combination provides a good balance of strength and durability to the felt with relatively little marking. Typically, the felt is constructed by flat weaving the duplex fabric, endless weaving the single layer fabric, joining the duplex fabric with a pin as described above, overlaying the single layer fabric over the duplex fabric, needling both fabric layers with batt to form machine side and paper side batt layers, removing the pin from the double layer fabric and cutting the batt layers and the single layer fabric at the seam to form a flat structure. Once at the paper mill, the felt is installed on the papermaking machine by inserting a new, typically thinner and more flexible pin into the duplex fabric layer.

This press felt construction has at least one significant shortcoming. When the single layer fabric is cut, its yarns tend to fray somewhat at the cut. Thus, when the felt is installed and operated on the paper machine, the frayed ends of the finer mesh single layer fabric can interfere with the manner in which the cut portion of the batt layer (which is often a flap of batt layer material) overlays the base fabric. As such, paper formed with such a felt can have an inconsistent appearance and be more susceptible to breaking on the paper machine due to the presence of the seam of the felt. One approach to this problem is offered in International Application 1200017433 (No. PCT/US98/19850) which discusses a press felt in which a band of cross machine direction yams formed of a "low melt" material is included at the seam of the single layer fabric. The low melt material can soften somewhat during heat-setting of the fabric, which can induce the cross machine direction yarns to agglomerate somewhat and reduce fraying.

### Summary of the Invention

In view of the foregoing, it is an object of the present invention to provide a press felt having a laminated base fabric with a reduced tendency for the fraying of yarns at the base fabric seam.

It is also an object of the present invention to provide such a press felt at a relatively low cost.

It is a further object of the present invention to provide a method for constructing such a press felt.

These and other objects are satisfied by the present invention, which is directed to a press felt that can have a reduced tendency to fray at the seam cut. The press felt according to claim 1 comprises: a paper side batt layer; a machine side batt layer; and a base fabric layer sandwiched between the paper side batt layer and the machine side batt layer. The base fabric layer comprises a first fabric and a second fabric. The first fabric includes machine direction yarns and cross machine direction yarns interwoven with the machine direction yarns. The first fabric has first and second ends with loops, wherein the loops of the first end are interdigitated with the loops of the second end, and the loops of said first and second ends receive a pin to form the first fabric into an endless belt having a seam. The second fabric is formed into an endless belt overlying the first fabric and includes machine direction yarns and cross machine direction yarns interwoven with the machine direction yarns, wherein the machine direction yarns are formed of a low melt material. In this configuration, the low melt machine direction yarns of the second fabric may have a reduced tendency to fray at the seam cut during prolonged operation.

Another aspect of the present invention is a method of constructing a papermaker's press felt according to claims 10 to 18.

### Brief Description of the Drawings

**Figure 1** is a schematic illustration of the press section of a paper machine employing a press felt of the present invention.
**Figure 2** is an enlarged partial cutaway perspective view of the press felt of **Figure 1.**
**Figure 3** is a greatly enlarged side section view of the press felt of **Figure 1.**
**Figure 4A** is a greatly enlarged partial perspective view of the pin seam of the press felt of **Figure 1** in a joined condition.
**Figure 4B** is an enlarged partial perspective view of the pin seam of **Figure 4A** in an unjoined position.
**Figure 5** is a schematic representation of a process for constructing the press felt of **Figure 1**.

### Detailed Description of the Invention

The present invention now will be described more fully hereinafter with reference to the accompanying drawings, in which preferred embodiments of the invention are shown and described. This invention may, however, be embodied in many different forms and should not be construed as limited to the embodiments set forth herein; rather, these embodiments are provided so that this disclosure will be thorough and complete, and will fully convey the scope of the invention to those skilled in the art. Like numbers refer to like components throughout. Components and layers may be exaggerated for clarity.

As used herein, the terms "machine direction" (MD) and "cross machine direction" (CMD) refer, respectively, to a direction aligned with the direction of travel of the papermakers' fabric on a papermaking machine, and a direction parallel to the fabric surface and transverse to the direction of travel. Also, both the flat weaving and endless weaving methods described hereinabove are well known in the art, and the term "endless belt" as used herein refers to belts made by either method.

Referring now to the drawings, a papermaking machine press section, designated broadly at **10,** is illustrated in **Figure 1**. The press section 10 includes a press felt **14** that is installed upon and conveyed by a set of rollers **12.** In its travel, the felt **14** travels over a press roll **15.** An opposed press **roll 17** is positioned to, in conjunction with the felt **14** and press roll **15,** form a nip **N** between the press rolls **15.**

In operation, a paper web **P is** conveyed from a forming section **16** through the nip **N** formed by the press rollers **15, 17,** wherein pressure is applied to the paper web **P** by the press rolls **15, 17.** The pressure forces moisture from the paper web **P** that is absorbed by the felt **14.** As the felt **14** is conveyed around its roller set **12**, moisture is removed therefrom, and the felt 1**4** is conditioned by one or more suction boxes 20.

**Figures 2** and **3** illustrate an enlarged section of the felt **14.** As can be seen in **Figure 2,** the felt **14** includes a laminated base fabric layer **22** which comprises two separate fabrics: namely, a lower fabric layer comprising a duplex fabric **24** and an upper fabric layer comprising a single layer fabric **36.** The duplex fabric **24** includes two sets of machine direction yarns 26 and one set of cross machine direction yarns **28** interwoven with the machine direction yarns **26.** The duplex fabric **24** is woven in a flat weave process; thus, in a flat condition, the duplex fabric **24** has two free ends **29a, 29b,** one of which **(29a)** includes loops **30** (formed by machine direction yarns **26),** and the other of which **(29b)** includes loops **32** formed by machine direction yarns **26.** When the duplex fabric **24** is in an endless condition such as that illustrated in **Figures 2** and **3,** the loops **30, 32** are positioned in interdigitated fashion, and a pin **34** is inserted through the loops 30, **32** to join the ends **29a, 29b** of the duplex fabric **24** (see **Figures 4A** and **4B).** This fabric can be flat woven in a process such as that disclosed in U.S. Patent No. 5,476,123 to Rydin.

Those skilled in this art will recognize that other types of fabrics can be employed as the lower fabric layer of the base fabric layer 22 in the manner of the duplex fabric 24, including single layer fabrics, other duplex fabrics, and triplex fabrics (i.e., those having two sets of machine direction yarns and two sets of cross machine direction yarns). Virtually any weave pattern known to those skilled in this art, such as the illustrated plain weave, twills, satins, and the like, can be used for this fabric layer. The lower fabric layer will typically, but not always, have a mesh that is somewhat more coarse than that of the upper fabric layer, it is preferred that the mesh of the lower fabric layer be between about 30 to 50 machine direction yarns and 50 to 100 cross machine direction yarns per inch. The lower fabric layer should have the aforementioned loops **30, 32** at its ends **29a, 29b** to enable it to be joined into an endless belt with the pin **34.** The construction of the loops 30, 32 and pin 34 are known to those skilled in this art and need not be described in detail herein; exemplary loop and pin constructions are described in U.S. Patent Nos. 4,737,241 and 4,764,417 to Gulya.

Referring again to **Figures 2** and **3,** the single layer fabric **36** comprises machine direction yarns 38 interwoven with cross machine direction yarns **40** in a plain weave pattern. The machine direction yarns **38** are formed of a low melt material that differs in composition from the material employed with the cross machine direction yarns **40** and the yarns of the duplex fabric **24.** As used herein, the term "low melt" means that the yarns have a lower melting point than at least the cross machine direction yarns **40** of the upper fabric 36, and in many instances than the other yarns of both the upper and lower fabric layers. The melting point of the low melt yarns is preferably at least 25°C lower than that of the machine direction yarns **26** of the lower fabric layer 24. Exemplary low melt materials to be employed as machine direction yarns **38** include nylons (including nylon 6, nylon 6-6, nylon 6-10, nylon 6-12 and nylon 12, and blends and copolymers thereof), polyesters and copolymers thereof and polypropylene and copolyiners thereof. It is preferred that the low melt material have a melting point of between about 130 and 200°C.

Those skilled in this art will recognize that other types of fabrics can be employed as the upper fabric layer of the base fabric layer 22 in the manner of the single layer fabric 36, including other single layer fabrics, duplex fabrics, and triplex fabrics. Virtually any weave pattern known to those skilled in this art, such as the illustrated plain weave, twills, satins, and the like, can be used for this fabric layer. The mesh of the upper fabric layer may vary from between about 16 to 100 machine direction yarns and 16 to 100 cross machine direction yarns per inch, but typically the mesh will be somewhat finer than that of the lower fabric layer. Those skilled in this art will also recognize that, although it may be preferred for cost reasons to employ low melt yarns as machine direction yarns 38 only, low melt yarns can also be used as the cross machine direction yarns 40 of for some or all of the single layer fabric 36, or even as the machine direction yarns 26 or cross machine direction yarns of the duplex fabric 24.

Illustratively and preferably, the single layer fabric 36 includes a band 42 that includes no cross machine direction yarns 40. The band 42 should overlie the pin 34 of the duplex fabric 24. The band 42 is approximately 2 to 12 inches with 8 inches being preferred in length (i.e., the band 42 extends approximately 4 inches on either side of the pin 34). The presence of the band 42 eliminates CMD yarns that might otherwise fray in the seam area.

Preferably, the single layer fabric 36 is woven in a flat weaving process that produces a fabric with two free ends. The single layer fabric 36 is formed into an endless belt through a joining process such as heat welding, which forms a weld line 46, although other methods of joining known in the art may also be employed. Alternatively, the single layer fabric 36 can be woven in an endless process so that the band 42 is formed during weaving.

The form of the yarns employed in the lower and upper fabric layers of the base fabric layer 24 can vary, depending upon the desired properties of the final press felt. For example, the yarns may be multifilament yarns, monofilament yarns, twisted or cabled multifilament or monofilament yarns, spun yarns, or any combination thereof. Also, the materials from which the "non-low melt" yarns employed in the fabric layers are formed may be those commonly used in press felts, such as nylon, cotton, wool, polypropylene, polyester, aramid, polyamide, or the like, and blends and combinations thereof.

Referring again to **Figures 2** and **3**, the felt 14 also includes scrim sheets **44a, 44b, 44c.** The scrim sheet **44a** is positioned between the double layer fabric 24 and the single layer fabric 36. The scrim sheet 44b is positioned directly beneath the double layer fabric 24. The scrim layer 44c is positioned directly above the single layer fabric 36. The scrim sheets 44a, 44b, 44c overlie the seam area of the felt 14, typically extending between about 4 to 10 inches on either side of the seam formed by the pin 34. Typically, the scrim sheets 44a, 44b, 44c comprise a non-woven, porous low melt nylon fabric.

Still referring to Figures 2 and 3, the felt 14 also includes two batt layers: a machine side batt layer 50 and a paper side batt layer 52. Illustratively and preferably, these batt layers 50, 52 are attached to the base fabric layer 22 through a needling process, although other attachment techniques, such as heat bonding and adhesives, can also be used with the present invention. An exemplary needling process is illustrated and described in co-assigned and co-pending U.S. Patent Application No. 09/359,213, the disclosure of which is hereby incorporated herein by reference in its entirety.

The machine side and paper side batt layers **50, 52** should be formed of material, such as a synthetic fiber like acrylic, aramid, polyester, or nylon, or a natural fiber such as wool, that assists in wicking water away from the base fabric layer **22**. Preferred materials for the batt layers **50, 52** include polyamide, polyester and blends thereof. The weight and thickness of the batt layers **50, 52** can vary, although it is preferably that the ratio of batt weight to fabric weight is about between about 0.5 and 2.0, with 1.0 being more preferred. Also, in some embodiments, it may be desirable to have additional batt layers or to omit either or both of the batt layers **50, 52.** Notably, the machine side belt layer 50 has an open area 50 below the pin 34 in which batt has been removed (Figure 3).

The felt 14 also includes a seam cut 48. The seam cut 48 extends through the paper side batt layer 52, the single layer fabric 36, and the machine side batt layer 50. Illustratively and preferably, the seam cut 48 is made at an angle of between about 30 and 80 degrees to the plane of the base fabric layer 22, and a flap 52a is formed by loosening the portion of the paper side batt layer 52 adjacent the seam cut 48. This process is described in detail in the aforementioned U.S. Patents to Gulya and Lilja. Of course, no cut is necessary for the duplex fabric 24, as the pin 34 can simply be removed to enable the ends 29a, 29b of the duplex fabric 24 to be separated.

**Figure 5** illustrates an exemplary manufacturing process for the felt 14. Initially, the duplex fabric 24 is flat woven such that machine direction loops 30, 32 are created on the ends **29a, 29b.** A pin 60 (which is typically larger and less flexible than the pin 34 described above) is inserted through the loops 30, 32 (as they are interdigitated) to join them and thereby form the duplex fabric 24 into an endless belt. Separately, the single layer fabric 36 is woven in a flat weaving or endless weaving process. If flat woven, the single layer fabric 36 is formed into an endless belt with a heat welding process, such as one that employs heat or ultrasonic radiation. The single layer fabric 36 is then positioned to overlie the duplex fabric 24 such that the band 42 that lacks cross machine direction yarns overlies the pin 34, the scrim sheets 44a, 44b, 44c are positioned over the seam area, and the machine side and paper side batt layers 50, 52 are needled to the base fabric layer 22 (the open area 50a is typically created by removing fiber with a brush and tweezers).

Once the batt layers 50, 52 have been added, the entire felt 14 is then heat treated at a temperature sufficient to cause softening of the machine direction yarns 38 formed of low melt material without unduly softening the other yarns of the base fabric 22. Typically, the heat treatment is carried out at a temperature of between about 130° to 200° C. The pin 60 is then removed, and the seam cut 48 is formed with blades or other cutting devices through the paper side batt layer 52 and the single layer fabric 36. The felt 14 can then be shipped in its flat form to a paper mill, where the pin 34 can be inserted into the machine direction loops 30, 32 as the felt 14 is installed on the upper rolls 12.

Importantly, when the seam cut 48 is made, the yarns of the single layer fabric 36, and in particular the machine direction yarns 38, can have a far lower tendency to fray than the fabrics of prior art felts. This reduced fraying is the result of the inclusion of the low melt machine direction yarns 38. As described, during the heat treatment of the felt 14, the softening of the low melt machine direction yarns 38 causes the agglomeration of the machine direction yarns 38 and the fibers of the paper side batt layer 52. As a result, the flap 52a adjacent to the seam cut 48 can lay uniformly, even during operation, which has not always been the case for prior art fabrics.

The invention will now be more particularly described in the following non-limiting example.

### EXAMPLE

A press felt was constructed according to the following parameters

| | **MD yarns** | | **CMD yarns** | | **Mesh Count** |
|---|---|---|---|---|---|
| **Base Fabric Layer** | **Size (inches)** | **Material** | **Size (inches)** | **Materials** | |
| Duplex Layer | 0.015 | Nylon | 0.415 | Nylon | 40x48 |
| Single Layer* | 0.014. | Nylon | 0.008 | Nylon | 40x24 |

| | | | | | |
|---|---|---|---|---|---|
| * The single layer fabric was woven without CMD yarns in a 8 inch wide band that was positioned directly over the pin seam of the duplex fabric. | | | | | |

| **Batt Layers** | **Material** | **Weight (g/m**^{**2**}**)** |
|---|---|---|
| Machine Side | Nylon staple | 150 |
| Paper Side | Nylon staple | 780 |

### Heat Treatment: 3 minutes at 175°C.

The resulting press felt successfully produced linerboard paper. ,

The foregoing is illustrative of the present invention and is not to be construed as limiting thereof. Although exemplary embodiments of this invention have been described, those skilled in the art will readily appreciate that many modifications are possible in the exemplary embodiments without materially departing from the novel teachings and advantages of this invention. Accordingly, all such modifications are intended to be included within the scope of this invention as defined in the claims. The invention is defined by the following claims.

## Claims

1. A papermaker's press felt comprising:
a paper side batt layer;
a machine side batt layer; and
a base fabric layer sandwiched between said paper side batt layer and said machine side batt layer, said base fabric layer comprising a first fabric and a second fabric;
said first fabric including machine direction yarns and cross machine direction yarns interwoven with said machine direction yarns, said first fabric having first and second ends with loops, said loops of said first end being interdigitated with said loops of said second end, said loops of said first and second ends receiving a pin to form said first fabric into an endless belt having a seam;
said second fabric formed into an endless belt overlying said first fabric and including machine direction yarns and cross machine direction yarns interwoven with said machine direction yarns, wherein said machine direction yarns are formed of low melt material.

2. The papermaker's press felt defined in claim 1, wherein said second fabric includes a band overlying said seam of said first fabric that has no cross machine direction yarns.

3. The papennaker's press felt defined in claim 1, said paper side batt layer and said machine side batt layer are needled to said base fabric layer.

4. The papermaker's press felt defined in claim 1, wherein said first fabric comprises a duplex fabric.

5. The papermaker's press felt as defined in claim 1, wherein said second fabric comprise a single layer fabric.

6. The papermaker's press felt as defined in claim 1, wherein said low melt material is selected from a group consisting of: nylon and nylon copolymer.

7. The papermaker's press felt defined in claim 1, wherein said first fabric layer forms a coarser mesh than said second fabric.

8. The papermaker's press felt as defined in claim 1, wherein each of said paper side batt layer, said machine side batt layer and said second fabric includes a cut corresponding to said first fabric seam to enable said press felt to take a flat condition upon removal of said pin.

9. The papermaker's press felt defined in claim 8, wherein said cut is oriented at an angle of between about 30 and 80 degrees relative to the plane of the base fabric layer.

10. A method of constructing a papermaker's press felt, said method comprising the steps of:
interweaving machine direction yarns and cross machine direction yarns to form a first fabric, said first fabric having first and second ends with loops;
positioning the loops of said first and second ends of said first fabric in interdigitated relationship;
inserting a pin into said loops to form a seam that joins the first and second ends of said first fabric, thereby forming said first fabric into an endless belt;
interweaving machine direction yarns and cross machine direction yarns to form a second fabric, wherein said machine direction yarns are formed of a low melt material;
attaching said second fabric to said first fabric ;
heating said low melt material to cause said low melt material to soften; and
cutting a seam through said low melt material that corresponds to said seam of said first fabric.

11. The method defined in claim 10, further comprising the step of attaching a first batt layer to overlie said second fabric layer.

12. The method defined in claim 11, wherein said cutting step further comprises cutting said first batt layer to form a seam therein.

13. The method as defined in claim 11, further comprising the step of attaching a second batt layer to underlie said fist fabric layer.

14. The method defined in claim 13, wherein said cutting step further comprises cutting said second batt layer to form a seam therein.

15. The method defined in claim 10, further comprising the step of removing the pin from said first fabric after said heating step and prior to said cutting step.

16. The method defined in claim 10, wherein said heating step comprises heating the low melt material at a temperature of between about 130°C and 200°.

17. The method defined in claim 10, wherein said step of intenveaving said second fabric comprises flat-weaving said second fabric.

18. The method defined in claim 10, further comprising the step of heat welding said second fabric to join ends thereof and thereby form said second fabric into an endless batt.

## Patentansprüche

1. Papiermaschinenpressfilz, Folgendes umfassend:
eine papierseitige Fasermattenschicht;
eine maschinenseitige Fasermattenschicht; und
eine Grundgewebeschicht, die sandwichartig zwischen der papierseitigen Fasermattenschicht und der maschinenseitigen Fasermattenschicht eingeschlossen ist, wobei die Grundgewebeschicht ein erstes Gewebe und ein zweites Gewebe umfasst;
wobei das erste Gewebe Maschinenrichtungsgarne und Quermaschinenrichtungsgarne enthält, die mit den Maschinenrichtungsgarnen verwebt sind, wobei das erste Gewebe erste und zweite Enden mit Schlingen aufweist, wobei die Schlingen des ersten Endes mit den Schlingen des zweiten Endes ineinandergreifend sind, wobei die Schlingen der ersten und zweiten Enden einen Dorn aufnehmen, um das erste Gewebe zu einem Endlosband mit einer Verbindungsnaht auszubilden;
wobei das zu einem Endlosband ausgebildete zweite Gewebe über dem ersten Gewebe liegt und Maschinenrichtungsgarne und Quermaschinenrichtungsgarne enthält, die mit den Maschinenrichtungsgarnen verwebt sind, wobei die Maschinenrichtungsgarne aus Material mit niedrigem Schmelzpunkt bestehen.

2. Papiermaschinenpressfilz nach Anspruch 1, wobei das zweite Gewebe ein über der Verbindungsnaht des ersten Gewebes liegendes Band enthält, das keine Quermaschinenrichtungsgarne aufweist.

3. Papiermaschinenpressfilz nach Anspruch 1, wobei die papierseitige Fasermattenschicht und die maschinenseitige Fasermattenschicht an der Grundgewebeschicht angenäht sind.

4. Papiermaschinenpressfilz nach Anspruch 1, wobei das erste Gewebe ein Duplexgewebe umfasst.

5. Papiermaschinenpressfilz nach Anspruch 1, wobei das zweite Gewebe ein Einschichtgewebe umfasst.

6. Papiermaschinenpressfilz nach Anspruch 1, wobei das Material mit niedrigem Schmelzpunkt aus einer Gruppe ausgewählt ist, die besteht aus: Nylon und Nyloncopolymer.

7. Papiermaschinenpressfilz nach Anspruch 1, wobei die erste Gewebeschicht ein gröberes Maschengitter bildet als das zweite Gewebe.

8. Papiermaschinenpressfilz nach Anspruch 1, wobei die papierseitige Fasermattenschicht, die maschinenseitige Fasermattenschicht und das zweite Gewebe jeweils einen der Verbindungsnaht des ersten Gewebes entsprechenden Einschnitt enthält, damit der Pressfilz beim Entfernen des Dorns einen flachen Zustand annehmen kann.

9. Papiermaschinenpressfilz nach Anspruch 8, wobei der Einschnitt in einem Winkel von ca. 30 bis 80 Grad bezüglich der Ebene der Grundgewebeschicht ausgerichtet ist.

10. Verfahren zum Aufbauen eines Papiermaschinenpressfilzes, wobei das Verfahren die folgenden Schritte umfasst:
Verweben von Maschinenrichtungsgarnen und Quermaschinenrichtungsgarnen, um ein erstes Gewebe auszubilden, wobei das erste Gewebe erste und zweite Enden mit Schlingen aufweist;
Anordnen der Schlingen der ersten und zweiten Enden des ersten Gewebes in ineinandergreifendem Verhältnis;
Einsetzen eines Dorns in die Schlingen, um eine Verbindungsnaht zu bilden, die die ersten und zweiten Enden des ersten Gewebes miteinander verbindet, wodurch das erste Gewebe zu einem Endlosband ausgebildet wird;
Verweben von Maschinenrichtungsgarnen und Quermaschinenrichtungsgarnen, um eine zweites Gewebe auszubilden, wobei die Maschinenrichtungsgarne aus einem Material mit niedrigem Schmelzpunkt bestehen;
Befestigen des zweiten Gewebes am ersten Gewebe:
Erhitzen des Materials mit niedrigem Schmelzpunkt, um es weich werden zu lassen; und
Einschneiden einer Verbindungsnaht durch das Material mit niedrigem Schmelzpunkt, die der Verbindungsnaht des ersten Gewebes entspricht.

11. Verfahren nach Anspruch 10, darüber hinaus den Schritt umfassend, eine erste Fasermattenschicht so anzubringen, dass sie über der zweiten Gewebeschicht liegt.

12. Verfahren nach Anspruch 11, wobei der Einschneideschritt darüber hinaus umfasst, die erste Fasermattenschicht einzuschneiden, um eine Verbindungsnaht darin auszubilden.

13. Verfahren nach Anspruch 11, darüber hinaus des Schritt umfassend, eine zweite Fasermattenschicht so anzubringen, dass sie unter der ersten Gewebeschicht liegt.

14. Verfahren nach Anspruch 13, wobei der Einschneideschritt darüber hinaus umfasst, die zweite Fasermattenschicht einzuschneiden, um eine Vrebindungsnaht darin auszubilden.

15. Verfahren nach Anspruch 10, darüber hinaus den Schritt umfassend, den Dorn nach dem Erhitzungsschritt und vor dem Einschneideschritt aus dem ersten Gewebe zu entfernen.

16. Verfahren nach Anspruch 10, wobei der Erhitzungsschritt umfasst, das Material mit niedrigem Schmelzpunkt auf eine Temperatur von ca. 130°C bis 200°C zu erhitzen.

17. Verfahren nach Anspruch 10, wobei der Schritt des Verwebens des zweiten Gewebes umfasst, das zweite Gewebe flachzuweben.

18. Verfahren nach Anspruch 10, darüber hinaus den Schritt des Warmverschweißens des zweiten Gewebes umfassend, um dessen Enden zu verbinden und dadurch das zweite Gewebe zu einer Endlosfasermatte auszubilden.

## Revendications

1. Feutre de presse de machine à papier comprenant :
une couche côté papier de tapis en fibre ;
une couche côté machine de tapis en fibre ; et
une couche de tissu de base prise en sandwich entre ladite couche côté papier de tapis en fibre et ladite couche côté machine de tapis en fibre, ladite couche de tissu de base comprenant un premier tissu et un deuxième tissu ;
ledit premier tissu comprenant des fils dans la direction de la machine et des fils dans la direction transversale de la machine tissés avec lesdits fils dans la direction de la machine, ledit premier tissu ayant des premières et deuxièmes extrémités comportant des boucles, lesdites boucles de ladite première extrémité interpénétrant lesdites boucles de ladite deuxième extrémité, lesdites boucles des premières et deuxièmes extrémités recevant une épingle pour former ledit premier tissu en une bande sans fin ayant une jonction ;
ledit deuxième tissu formé en une bande sans fin se superposant au dit premier tissu et incluant des fils dans la direction de la machine et des fils dans la direction transversale de la machine tissés avec lesdits fils dans la direction de la machine, lesdits fils dans la direction de la machine étant formés en un matériau à basse température de fusion.

2. Feutre de presse de machine à papier selon la revendication 1, dans lequel le deuxième tissu comprend une bande se superposant à ladite jonction dudit premier tissu qui n'a pas de fils dans la direction transversale de la machine.

3. Feutre de presse de machine à papier selon la revendication 1, dans lequel ladite couche côté papier de tapis en fibre et ladite couche côté machine de tapis en fibre sont aiguilletées avec ladite couche de tissu de base.

4. Feutre de presse de machine à papier selon la revendication 1, dans lequel ledit premier tissu comprend un tissu en couche double.

5. Feutre de presse de machine à papier selon la revendication 1, dans lequel ledit deuxième tissu comprend un tissu en couche simple.

6. Feutre de presse de machine à papier selon la revendication 1, dans lequel ledit matériau à basse température de fusion est choisi dans un groupe consistant de : nylon et copolymère de nylon.

7. Feutre de presse de machine à papier selon la revendication 1, dans lequel ladite première couche de tissu forme une maille plus grossière que ledit deuxième tissu.

8. Feutre de presse de machine à papier selon la revendication 1, dans lequel chacun parmi ladite couche côté papier de tapis en fibre, ladite couche côté machine de tapis en fibre et ledit deuxième tissu comprend une coupe correspondant à ladite jonction de premier tissu pour autoriser ledit feutre de presse à adopter un état plat lorsqu'on enlève ladite épingle.

9. Feutre de presse de machine à papier selon la revendication 8, dans lequel ladite coupe est orientée selon un angle d'environ 30 à 80 degrés par rapport au plan de ladite couche de tissu de base.

10. Méthode pour construire un feutre de presse de machine à papier, ladite méthode comprenant les étapes de :
tisser des fils dans la direction de la machine et des fils dans la direction transversale de la machine pour former un premier tissu, ledit premier tissu ayant des premières et des deuxièmes extrémités avec des boucles ;
positionner en relation d'interpénétration les boucles desdites premières et deuxièmes extrémités dudit premier tissu ;
insérer une épingle dans lesdites boucles pour former une jonction qui joint les premières et deuxièmes extrémités dudit premier tissu, formant ainsi ledit premier tissu en une bande sans fin ;
tisser des fils dans la direction de la machine et des fils dans la direction transversale de la machine pour former un deuxième tissu, dans lequel lesdits fils dans la direction de la machine sont formés en un matériau à basse température de fusion ;
attacher ledit deuxième tissu audit premier tissu ;
chauffer ledit matériau à basse température de fusion de façon à ce que ledit matériau à basse température de fusion se ramollisse ; et
couper une jonction à travers ledit matériau à basse température de fusion qui correspond à ladite jonction dudit premier tissu.

11. La méthode selon la revendication 10, comprenant en outre l'étape d'attacher une première couche de tapis en fibre en superposition à ladite deuxième couche de tissu.

12. La méthode selon la revendication 11, dans laquelle ladite étape de coupe comprend en outre la coupe de ladite première couche de tapis en fibre pour y former une jonction.

13. La méthode selon la revendication 11, comprenant en outre l'étape d'attacher une deuxième couche de tapis en fibre en sous-couche à ladite première couche de tissu.

14. La méthode selon la revendication 13, dans laquelle ladite étape de coupe comprend en outre la coupe de ladite deuxième couche de tapis en fibre pour y former une jonction.

15. La méthode selon la revendication 10, comprenant en outre l'étape d'enlever l'épingle du premier tissu après ladite étape de chauffage et avant ladite étape de coupe.

16. La méthode selon la revendication 10, dans laquelle ladite étape de chauffage comprend le chauffage du matériau à basse température de fusion à une température d'environ 130 °C à 200 °C.

17. La méthode selon la revendication 10, dans laquelle ladite étape de tissage dudit deuxième tissu comprend le tissage à plat dudit deuxième tissu.

18. La méthode selon la revendication 10, comprenant en outre l'étape de soudage à chaud dudit deuxième tissu pour en joindre les extrémités et former ainsi le deuxième tissu en un tapis en fibre sans fin.
